

April 2, 1929.

L. H. MARSHALL

1,707,529

METALLURGICAL PROCESS AND PRODUCT

Filed Jan. 19, 1925

4 Sheets-Sheet 1



FIG. 1.

Inventor

witness:

H. J. Stromberger

By

James J.

Attorney

LESLIE H. MARSHALL

April 2, 1929.

L. H. MARSHALL

1,707,529

METALLURGICAL PROCESS AND PRODUCT

Filed Jan. 19, 1925

4 Sheets-Sheet 2



FIG. 2.

Inventor

Witness:

H. J. Stromberger

LESLIE H. MARSHALL

H. G.

Gause

Attorney

April 2, 1929.

L. H. MARSHALL

1,707,529

METALLURGICAL PROCESS AND PRODUCT

Filed Jan. 19, 1925

4 Sheets-Sheet 3



FIG. 3.

Inventor

witness:

*H. J. Stromberger*

By

LESLIE H. MARSHALL

*James C.*

Attorney

April 2, 1929.

L. H. MARSHALL

1,707,529

METALLURGICAL PROCESS AND PRODUCT

Filed Jan. 19, 1925

4 Sheets-Sheet 4



FIG. 4.



FIG. 5.

witness:

H. J. Stromberger

By

LESLIE H. MARSHALL

Greenlee

Attorney

## UNITED STATES PATENT OFFICE.

LESLIE H. MARSHALL, OF MANSFIELD, OHIO, ASSIGNOR TO THE OHIO BRASS COMPANY, OF MANSFIELD, OHIO, A CORPORATION OF NEW JERSEY.

## METALLURGICAL PROCESS AND PRODUCT.

Application filed January 19, 1925. Serial No. 3,375.

My invention relates to malleableized cast iron, and the manufacture of the same. Malleableized cast iron is the result of changing the combined carbon of a casting into a free or graphitic carbon whereby the original casting, which is very hard and brittle, becomes soft and ductile, easily machined and even bent under satisfactory conditions.

The production of malleableized cast iron 10 may be said to comprise two principal steps—first, that of casting the desired article out of hard or white iron in which the carbon is in a chemically combined condition and—second, annealing the hard iron 15 casting, that is, subjecting the hard, brittle casting to a proper heat treatment whereby the combined carbon will be converted into a free or graphitic carbon.

The production of malleableized cast iron 20 is an old art, but under the present process or processes for producing malleableized cast iron the physical properties are not uniform and reliable and there is no assurance they can be zinc-coated, as by the hot dipped and 25 Sherardizing processes, etc. without embrittlement.

My invention has particularly to do with the annealing cycle and possesses several advantages, namely; the production of—

30 A product which will be uniform as to its physical properties and hence reliable,

35 A product which for any given composition possesses a relatively high impact value as measured by an impact machine,

40 A product which can be given a rust proofing coating, (such as hot galvanizing or Sherardizing) under heat without embrittlement of the casting,

45 A product which can be produced in a shorter time than a product subjected to the present commercial process or processes of annealing,

50 A product having a uniform distribution of its ingredients and hence homogeneous.

45 Referring to the drawings:

55 Figs. 1, 2, and 3, show certain curves employed in describing my invention and in differentiating it from the prior art, as will hereinafter more clearly appear.

50 Fig. 4 is a perspective view of a furnace which may be employed in carrying my invention into practice.

55 Fig. 5 is a section on the line 5—5 of Fig. 4. As now carried out, generally the process

of malleableizing cast iron consists in producing a casting which consists principally of iron, carbon, silicon, phosphorus, sulphur and manganese. The carbon is in a chemically combined state and forms a compound with the iron known as cementite and such iron is very hard and brittle and the object of malleableizing is to render the iron soft and ductile and this is brought about by heating the hard iron casting to a temperature somewhat above its critical temperature (about 1400° F., but which varies with the chemical composition of the iron) and usually not above 1700° F. to 1750° F. as it is difficult to maintain the refractory walls of the heating ovens and the quality of the iron produced is liable to be affected with too high a temperature. The time the iron is subjected to a temperature above the critical depends upon the temperature and composition, and the higher the temperature the less the time required. Under this heating all the combined carbon is changed to graphitic carbon with the exception of about .8% which remains as combined carbon. To still further transform the combined carbon, the temperature of the iron is allowed to drop slowly, possibly at the rate of approximately 5° F. to 12° F. per hour until a temperature of approximately 1200° F. to 1300° F. is reached, just below the critical, and during this drop in temperature the graphitization is completed or reaches an equilibrium, that is, all the remaining combined carbon has been transformed into free carbon with the exception of about .1% which remains as a combined carbon and is characteristic of malleableized cast iron. After the iron has cooled to 1200° F. or 1300° F. it is allowed to cool to room temperature or until it may be handled, but no consideration is given to the rate of cooling other than it is considered necessary to cool slowly.

60 I have found that the rate of cooling and the temperature from which the iron is cooled after graphitization is completed is of the utmost importance if an iron having the best properties is desired, and to the best of my knowledge, no thought has been given in the past to the last step in the annealing process, namely—cooling after graphitization.

65 It is well to state here that I have found that each composition of iron possesses its

own characteristics and these are clearly shown when different grades are subjected to comparative tests and therefore it is not possible to say that characteristics possessed by one grade of iron will apply to other grades, still in order to clearly disclose my invention I am obliged to refer to definite figures and limits in many cases, but it should not be considered that these will apply to all compositions of iron.

In Fig. 1 I have shown a set of curves to represent the four steps employed in the annealing or graphitizing of the hard iron and curve A represents the thermal cycles through which the iron passes when annealed in a furnace usually employed by malleable cast iron foundries. One of the usual methods of annealing is to place the hard iron castings in an inert packing material such as mill-scale or sand contained in pots or containers which are placed on the floor of the furnace, which is then brought up to the temperature desired, then held, then dropped slowly to a point below the critical temperature and then the furnace is opened and the content allowed to cool as it will. A complete cycle of 186 hours is shown in curve A and comprises 36 hours to bring the contents up to the preliminary graphitizing temperature of 1650° F. at which temperature it is held for 60 hours and then allowed to cool slowly at the rate of substantially 6.8° F. per hour to 1200° F. During this period of slow cooling the graphitizing will reach a state of equilibrium and the furnace doors are opened and the contents allowed to cool either to room temperature or until the pots may be handled conveniently. As the pots are packed in the furnace quite close and as the mass to cool is large, the castings in the pots farthest from the door cool much slower than the castings in the pots near the door hence there is not a uniform rate of cooling. In curve A, Fig. 1, the furnaces are shown as drawn at 24 hours after the doors are opened and if the castings near the door reach room temperature, the cooling will be at a rate of about 50° F. per hour, and if those at the rear of the furnace have cooled to 500° F. their rate of cooling will be much slower, about 30° F. per hour. As stated before, I have found the rate of cooling of the greatest importance, but the rate of heating the castings up to the maximum temperature is unimportant, the time, however, of holding at the maximum temperature and the rate of cooling to the temperature at which the furnace door is opened is important and has been recognized for a long time.

Malleableized cast iron made as above described is not uniform in its physical properties and is not of the highest quality for any given composition and it will not always hot-galvanize or lend itself to a heat treat-

ment within galvanizing temperatures without embrittling, and variations may take place in the iron from a single anneal or heat and these variations and lowered physical properties are, I find, due to improper cooling after graphitization has been completed or equilibrium has been reached.

In Fig. 2 I show a set of curves based upon impact values on two grades of commercial malleableized cast iron which had been subjected to the usual annealing process. The curves were produced by plotting impact values in per cent of that of the normal or commercial iron after the various samples had been machined to a standard size and heated to different temperatures from about 400° F. to 1472° F. and quenched in water at 175° F. The normal or 100% line represents the impact value of the untreated commercial iron produced according to the usual annealing process. The samples after being heated to the temperatures shown by the points on the curves and quenched in water at 175° F. were tested in an Izod impact machine which measured the resiliency in foot pounds and these readings were then reduced to per cent of the impact value of the normal or commercial iron.

These curves show that if normal commercial malleableized cast iron represented by these curves is heated to certain temperatures and then quenched that their resiliency will be less than before heating and cooling and the greatest loss in resiliency is through that range of temperature to which the iron would be subjected if hot galvanized, approximately 850° F. to 925° F. The curves also show that if the iron is heated to certain other temperatures and quenched that the resiliency is greater than the normal commercial product and in case of the C iron the resiliency is increased 50% by heating to about 1130° F. and quenching and in case of D iron the resiliency is increased about 15% by heating to about 1022° F. and quenching. I have found that iron heated to a temperature above that at which the curves cross the normal line and then quenched that such iron may be hot galvanized without embrittlement. This disclosure is set forth in my copending application Serial No. 633,789, filed April 21, 1923 (now Patent No. 1,553,907, granted September 15, 1925).

I have also found that some grades of regularly treated commercial malleableized cast iron may be heated up to a temperature above the crossing of its impact curve with the normal line, but below the critical temperature, and then cooled rapidly, as for instance, at a rate of about 6° F. of 7° F. per minute, that such treated iron will galvanize without embrittlement. The effect of cooling at such rate on a grade of iron from a

temperature of 1250° F. is represented by curve F, Fig. 3, and later referred to herein.

I have discovered, that if, when graphitization has been completed, the castings are 5 removed from the oven and quenched or cooled quickly, the entire heat will be uniform, the physical properties of the individual castings will be improved over those of the usual commercial castings and the 10 structure will be homogeneous, and they may be galvanized or subjected to heat within the galvanizing range without embrittlement and the time of the annealing process will be reduced by the amount of time allowed for 15 the product to cool under present operating conditions.

In Fig. 1 I have shown by the lines B<sup>1</sup> and B<sup>2</sup> the last step of annealing by my process when substituted for the last step as 20 shown by curve A and the reduction shown is about 24 hours. B<sup>1</sup> represents the castings drawn as soon as the graphitization has been completed and quenched in water, and B<sup>2</sup> represents the castings drawn at 25 once and cooled at a rate of about 6° F. to 7° F. per minute.

I find that the purer the hard iron is the slower it may be cooled in the last step of the annealing operation, as will be shown 30 later, but I have found that quenching or cooling quickly from about 1200° F. to 1300° F. will for any given composition produce a uniform grade of iron of best qualities and this method applies to all compositions usually employed.

It will be recognized that the A<sup>1</sup> step shown in Fig. 1 can be made as rapid as possible, also the A<sup>2</sup> and A<sup>3</sup> steps may be shortened from that shown so long as at each 40 step the proper amount of graphitization has been carried out, but whatever the A<sup>1</sup>, A<sup>2</sup> and A<sup>3</sup> periods may be, by quenching for the A<sup>4</sup> step the total annealing time may be shortened many hours from the present 45 process.

In carrying out my process with the ordinary furnace (see Figs. 4 and 5) the pots or containers 1 with the hard iron castings therein would be mounted on trucks 2 and run into the furnace on rails 3 and coupled together if two or more are placed end to end by the couplers 4. The furnace would, of course, be provided with a sand or other seal 5 to prevent the heat from affecting the 55 truck mountings and the rails. The furnace is then brought up to the required temperature by means of powdered coal, gas or oil heat through the ports 6 or by other means, and the time and temperature for the 60 A<sup>1</sup>, A<sup>2</sup> and A<sup>3</sup> steps manipulated according to a predetermined standard. When the A<sup>3</sup> step has been completed the furnace doors are opened and the trucks and castings withdrawn at once and dumped, preferably on 65 a grating conveniently located, which will

allow the packing material to sift through and expose the castings to the air and hence quench them more quickly, or the pots may be dumped on to a moving conveyance running through water and quenched or cooled 70 still more rapidly. Fig. 5 is a sectional view of Fig. 4 through the plane 5.

Tests made upon specimens of iron containing:

|            |       |    |
|------------|-------|----|
| Silicon    | 0.94  | 75 |
| Sulphur    | 0.063 |    |
| Manganese  | 0.35  |    |
| Phosphorus | 0.236 |    |
| Carbon     | 2.31  | 80 |

and using the Izod type of impact machine which measures the resiliency in foot pounds showed that the above iron when put through the first three steps of annealing and quenched in water when the third step 85 had been completed at about 1250° F. had an impact value of 11.5 foot pounds and when other specimens of the same composition and annealed at the same time and hence under the same conditions were 90 allowed to cool slowly at 8° F. per hour, such specimens showed an impact value of only 3.4 foot pounds. When the first samples above were subjected to the galvanizing process and then tested by the Izod machine 95 they showed 13.6 foot pounds and when the slowly cooled samples were galvanized and tested they showed only 1.0 foot pound. From these figures it will be noted that rapid cooling from 1250° F. has produced 100 a malleableized cast iron of 3.4 times the resiliency of an iron cooled slowly from 1250° F. and after galvanizing the resistance of the quickly cooled specimens was 13.6 times that of the slowly cooled specimens. 105

I also found that the temperature from which the specimens were cooled or quenched had an effect upon the impact value, as for instance, specimens of the same composition of iron as above when treated as above and 110 cooled slowly to 1050° F. and quenched from that temperature the impact value was 7.1 foot pounds and after galvanizing 9.0 foot pounds, and this same iron when cooled slowly to and quenched from 850° 115 F. the impact value was only 1.4 foot pounds and after galvanizing 1.1 foot pounds.

I have obtained similar variations to the above on other grades or compositions of 120 iron, all tending to show that the rate of cooling and the temperature from which the iron is cooled is important and varies with the composition of the iron, hence it is impossible to give figures which will apply to 125 all compositions of iron.

Along this line the curves shown in Fig. 3 will be of value. The compositions of the commercial iron vary considerably as to phosphorus, silicon and carbon and it will 130

be noted that there is a difference in the impact values when quenched in water from 1250° F. The impact values are plotted in percent of the water quenched value which cannot conveniently be shown on the curve as it is too far to the right.

Curve F shows that the iron it represents has practically reached its maximum resiliency when cooled at not less than about 7° F. per minute (420° F. per hour) from 1250° F. and that more rapid cooling does not increase the resiliency, as measured by the Izod machine, to a great extent.

Curve G shows that the iron it represents requires a cooling rate of at least 110° F. per minute to approximate the best results and to equal that secured on F iron when cooled at about 7° F. per minute, this iron should, therefore, be quenched in water from about 1250° F. to secure the greatest resiliency.

The impact test values were made after the specimens had been cooled or quenched at the rates shown from 1250° F. and then galvanized and show not only the effect of cooling rates on the two compositions of iron, but also the fact that different compositions may be given different treatments or rates of cooling, but that there is a minimum rate which, if decreased will give an iron of inferior quality. The curves also show that galvanizing the iron produced by my process does not embrittle the iron. The iron represented by the curve G is unusually high in phosphorus and silicon and requires much more rapid cooling than the iron represented by curve F and these and other tests show, and I have found by actual tests that for the average commercial grades of iron that if they are removed from the furnace at approximately 1200° F. or 1300° F. and shaken from the pots so that they will air cool, they will be free from a tendency to embrittle when galvanized.

In searching for a cause for the benefits derived from proper cooling from the final graphitization temperature, I have come to the conclusion that at some temperature below the critical temperature the impurities or other ingredients are uniformly dispersed throughout the mass. If allowed to cool slowly from this temperature, the impurities and other ingredients are given an opportunity to segregate along the crystalline boundaries thereby giving a non-homogeneous structure which is weak at some points and stronger at others, the result being an unreliable product and one which will not hot galvanize without danger of embrittlement, because these segregations are embrittled by the galvanizing treatment and offer an easy path to fracture. The greater the amount of impurities the greater the unreliability of the product under ordinary pro-

cesses of annealing, also the lower the impact value.

If on the other hand the iron at slightly below the critical temperature is suddenly quenched or cooled with sufficient rapidity the impurities and other ingredients which are uniformly distributed do not have time to segregate or collect in groups, but are held in a uniformly distributed state when the mass cools quickly or is quenched and hence we have a homogeneous mass with the ingredients distributed uniformly throughout the crystalline grains thereby giving a uniform and reliable product of the greatest resiliency value which that grade of iron is capable of and one which will hot galvanize without embrittlement.

Therefore, in carrying out my invention, after the product has cooled to a temperature at which graphitization has reached a state of final equilibrium and all the combined carbon has been graphitized except about 0.1%, and which temperature might be referred to as the equilibrium temperature, I quench the iron at such temperature or at some lower temperature at which the impurities are still in a homogeneous state of distribution, or I cool sufficiently rapid from such temperatures so as to prevent the impurities and other ingredients from segregating into groups or other non-homogeneous state throughout the mass.

My invention may be carried out to advantage in a continuous furnace kiln in which the pots of hard iron castings are placed on a truck and moved into a chamber at 1650° F. or other suitable temperature, and where they will come up to temperature in approximately 5 to 10 hours and they will remain under this temperature for the necessary time and then moved along to a second compartment where the temperature is lower and they will cool slowly at 8° F. per hour or much faster as found practical and until the graphitization process has been completed, and then the truck will be moved forward onto a grating and automatically dumped and the castings exposed to the atmosphere and air quenched or they may be dumped onto a conveyance moving through water to quench. Using a continuous kiln the cycles of time and temperature are shown by curve E on Fig. 1, and using the same values for E<sup>2</sup> and E<sup>3</sup> as for A<sup>2</sup> and A<sup>3</sup>, it will be seen that approximately 51 hours is saved in the process. The steps E<sup>2</sup> and E<sup>3</sup> may be shortened as much as the grade of iron and other conditions will permit in securing an equilibrium in graphitization of the iron.

Iron which has been treated as described from the graphitization temperature or other temperature as described may be hot galvanized without embrittlement of the

iron by applying the galvanizing process as is well known, consisting principally in cleaning the castings in dilute hydrochloric, sulphuric acid, etc. then subjecting them to a 5 bath of molten zinc and after shaking the surplus zinc from the castings either cool quickly or quench.

I have found that quenching malleable- 10 iron castings in water from a tempera- 10ture of approximately 1250° F. will prevent embrittlement of all compositions of iron of commercial value. Some compositions can be quenched in water from a lower tem- 15 perature than 1250° F. and will be immune 15 to embrittlement.

All compositions will give a high impact 20 value, when treated as herein described, such values depending upon the composition of the iron.

20 Some compositions may be quenched or cooled at a slower rate than others and still be immune from embrittlement.

The greater the impurities the faster the 25 rate of cooling should be and the higher 25 the temperature at which the rapid cooling is initiated (not to exceed the critical tem- 25 perature).

30 Apparently when the iron is at a certain temperature the impurities are uniformly dispersed therein and the iron should be cooled or quenched before the impurities have had an opportunity of segregating.

To practice my process it is not necessary 35 to always quench in water, as quenching in air will give the required results if the tem- 35 perature is sufficiently high and the castings not too large to cool sufficiently rapid, at least this is true of most compositions.

To produce satisfactory results it appears 40 from tests that iron should not be cooled slower than about 360° F. per hour, depending upon the composition, and from a tem- 40 perature at which the impurities are uni- 40 formly disseminated.

45 If the product is chilled after the impuri- 45 ties have begun to segregate the resulting product will be correspondingly inferior to a product chilled before segregation begins to take place.

50 Those skilled in the art know that the hard iron can be graphitized by bringing the castings to a temperature just below the critical temperature, about 1375° F., and holding it there for a protracted period of time, but 55 this is practical only with high silicon iron on account of the time required to bring about the equilibrium. Should this step be employed, however, then the next step should be to quench from that temperature as de- 60 scribed above.

It will also be recognized by those skilled 65 that after the preliminary graphitization above the critical temperature the castings may be cooled as rapidly as oven conditions will permit to a temperature just below the

critical temperature and then held at this temperature until the second stage of graphitization has been completed, and if now the castings are chilled, as I have herein de- 70 scribed, and before detrimental segregation of the impurities can take place, the bene- 70 ficial results herein described will be secured.

In the appended claims I use the word quenched, or quenching, to indicate air cool- 75 ing; or liquid cooling; or cooling in a fur- 75 nace but at a comparatively rapid rate such, for example, as would take place in a com- 80 paratively small or experimental furnace as distinguished from a large commercial fur- 80 nace, or by forcing cold air into the anneal- 80 ing furnace after the graphitization steps have been completed and forcing the hot air out and rapidly drawing off the heat from the castings.

In the appended claims I use the expres- 85 sions "carbon—combining temperature" and "critical temperature" synonymously. By "neutral temperature" I mean such tempera- 90 ture that if the iron is brought to a tempera- 90 ture below the critical temperature and not less than said "neutral temperature", and then cooled, it will not be embrittled, or in danger of embrittlement. These various ex- 95 pressions will be understood when considered in the light of the above disclosure and also 95 when considered in the light of the disclosure in my copending application Ser. No. 633,789 (now Patent No. 1,553,907).

In the specification of my said application Serial No. 633,789 (now Patent No. 1,553,- 100 907) and the specification of the present application two processes, among others, are taught. One of these two processes includes the following steps:—

(a) Raising the temperature of the iron 105 in the hard iron condition to a temperature above the critical or carbon-combining tem- 105 perature,

(b) Cooling the iron comparatively slowly to a temperature below the carbon- 110 combining temperature,

(c) Cooling the iron at a more rapid but still comparatively slow rate as by opening the door of a comparatively large furnace,

(d) Raising the temperature of the iron 115 to a temperature below the carbon-combining or critical temperature but above the neutral temperature; i. e., a temperature within the safety zone,

(e) Quenching the iron; i. e., plunging it 120 in liquid, cooling in air, or opening the doors of a small experimental furnace.

The other of the two processes referred to includes the following steps:

(a) Raising the temperature of the iron 125 in the hard iron condition to a temperature above the critical or carbon-combining tem- 125 perature,

(b) Cooling the iron comparatively slowly to a temperature below the carbon- 130

combining temperature but above the neutral temperature,

(e) Quenching the iron (i. e., plunging it in liquid, cooling in air, or opening the doors of a small experimental furnace) before its temperature has been allowed to drop below the neutral temperature.

All of the claims of the said Patent No. 1,553,907, cover the first of the two processes outlined above; some of the claims of the patent cover that process but not the second process; and others of the claims of the patent cover both processes. In the present application the claims cover the second of the two processes outlined above but not the first.

I claim:

1. The method of producing malleable cast iron comprising the steps of heating the iron to a temperature above the carbon-combining temperature, lowering the temperature of the iron to a temperature below the carbon-combining temperature, and then quenching the iron while its temperature is above and before its temperature has been allowed to drop below that which will cause the iron to be in danger of embrittlement.

2. The method of producing malleable cast iron comprising the steps of heating the iron to a temperature above the carbon-combining temperature, lowering the temperature of the iron to a temperature below the carbon-combining temperature, and then quenching the iron in liquid while its temperature is above and before its temperature has been allowed to drop below that which will cause the iron to be in danger of embrittlement.

3. The method of producing malleable cast iron comprising the step of heating the iron to a temperature above the carbon-

combining temperature, maintaining the iron at that temperature for a period dependent upon the composition of the iron and the temperature to which it has been raised, and cooling the iron to a temperature below the carbon-combining temperature, in accordance with the ordinary American commercial annealing operation, and then quenching the iron while its temperature is above and before its temperature has been allowed to drop below the neutral temperature.

4. The method of producing malleable cast iron comprising the steps of annealing the iron in the hard iron condition by subjecting the iron to such temperature for such time as to change the combined carbon into free or graphite carbon, then stabilizing the annealed iron by quenching it before its temperature has been allowed to drop below that which will cause the iron to be embrittled.

5. The method of producing rust-proof malleable cast iron which comprises the steps of heating the iron to a temperature above the carbon-combining temperature, maintaining the iron at that temperature for a period dependent upon the composition of the iron and the temperature to which it has been raised, and cooling the iron to a temperature below the carbon-combining temperature, in accordance with the ordinary American commercial annealing operation; quenching the iron while its temperature is above and before its temperature has been allowed to drop below the neutral temperature, and coating the iron with a rust-proofing material with the application of heat.

In testimony whereof I affix my signature.

LESLIE H. MARSHALL.